

Jan. 20, 1942.

F. KUHN ET AL

2,270,316

FINISH FOR WORKING SURFACE OF LAUNDRY IRONS AND THE LIKE

Filed July 7, 1941



FIG.1.

FIG.2.



FIG.3.



INVENTORS

FRANK KUHN

LAURENCE H. THOMAS

BY *Whittemore, Hullert & Belknap*

ATTORNEYS

## UNITED STATES PATENT OFFICE

2,270,316

FINISH FOR WORKING SURFACE OF  
LAUNDRY IRONS AND THE LIKE

Frank Kuhn, Detroit, and Laurence H. Thomas,  
Birmingham, Mich., assignors to American  
Electrical Heater Company, Detroit, Mich., a  
corporation of Michigan

Application July 7, 1941, Serial No. 401,354

5 Claims. (Cl. 38—93)

The invention relates to laundry irons and the like and has for its object reduction in the labor required for performance of work therewith.

In the manual operation of ironing, a considerable portion of the effort required is in overcoming the frictional resistance to the sliding of the iron over the surface operated upon. To reduce this resistance, it has been the practice to form the working surface of the laundry irons with a highly polished mirror-like finish. Also, in recent years it has been usual to plate the working surface with a metal differing from that forming the body of the iron, as, for instance, nickel or chromium. Where the latter material is used, it is customary to electrolytically deposit it upon an under surface of some other metal such as nickel, which under surface is first prepared by imparting thereto a mirror-like finish which is reproduced in the chrome plating.

Our invention is based on the discovery that frictional resistance due to the movement of the iron over the surface with which it is in contact is reduced by substituting for the mirror-like surface a surface less highly polished. It has been found by carefully conducted scientific tests that the frictional resistance measured by the force required to move the iron over the work can be reduced as much as fifty percent, when a dull finish is substituted for a mirror finish.

It has also been found that where the less highly polished surface is formed by abrasive material moved in one direction with respect to the iron, the friction will be less to movement in this direction than to a movement transverse thereto. Inasmuch as a laundry iron is usually manipulated by a movement longitudinally thereof, a surface having the microscopic lines therein extending longitudinally of the iron will have an advantage over one in which the lines extend in some other direction. While we do not fully understand the reason for such effect, experimental evidence has fully demonstrated the same.

Our invention therefore consists:

First, in a working surface for a laundry iron or the like which has a smooth but non-mirror-like character;

Second, in such a surface where the microscopic lines extend parallel to each other over the entire surface;

Third, in such a surface where the microscopic lines extend parallel to each other and longitudinally of the iron; and

Fourth, in the specific construction as herein-after set forth.

Inasmuch as the change in structure is microscopic, it cannot be exactly illustrated, but is represented more or less diagrammatically and exaggerated in the drawing, in which:

5 Fig. 1 is a bottom plan view of a laundry iron illustrating diagrammatically the character of the working surface thereof;

Fig. 2 is a rear end elevation of Fig. 1; and

Fig. 3 is a cross section illustrating on a magnified scale the character of both the under and the working surface of the iron.

As illustrated, A is a laundry iron of any suitable construction, and B is the bottom or sole plate thereof. The body of this plate may be formed of any suitable material such as iron or steel, which, after preliminary grinding, is provided with a fairly heavy electrolytic deposit C of some other metal such as nickel. The lower surface of this coating is then prepared, preferably by buffing with a soft fabric wheel and a suitable grade of abrasive. For the latter, emery or a similar abrasive may be used, of a grade between 120 and 400 grit, preferably 140. The buffing is effected by a movement of the buffing wheel relative to the sole plate, longitudinally of the latter, so that the effect will be to form parallel microscopic lines extending longitudinally of the iron. The prepared surface is then coated with an electrolytic deposit D of chromium, which is quite thin and conforms to the character of the under surface.

A laundry iron formed as above described will offer a greatly reduced frictional resistance to sliding movement over the surface that is being ironed, particularly where this movement is in a direction longitudinal with respect to the iron.

What we claim as our invention is:

1. In a laundry iron or the like, a sole plate provided with a metallic working surface having a substantially smooth but non-mirror-like characteristic formed by parallel microscopic lines extending in one direction thereacross.

2. In a laundry iron or the like, a sole plate provided with a non-mirror-like working surface with parallel microscopic lines extending in one direction thereacross corresponding to that produced by an abrasive of 140 grit.

3. In a laundry iron, a sole plate having a non-mirror-like working surface with parallel microscopic lines therein extending longitudinally of the iron.

4. In a laundry iron or the like, a sole plate having on its lower surface an electrolytic coating of another metal, said coating having its outer surface smooth but non-mirror-like and

with parallel microscopic lines extending longitudinally thereof, and a chromium electrolytic coating upon said first-mentioned coating having a corresponding surface.

5. In a laundry iron or the like, a sole plate having a non-mirror-like working surface cor-

responding to that produced by an abrasive between 120 and 400 grit and with parallel microscopic lines therein extending longitudinally of said sole plate.

FRANK KUHN.

LAURENCE H. THOMAS.